

Nov. 19, 1929.

H. M. NAUGLE, ET AL  
STRIPSHEET MANUFACTURE

1,736,324

Filed May 24, 1927

3 Sheets-Sheet 1



Fig. 1



Fig. 2



Fig. 3



Fig. 4

Inventors

H. M. Naugle  
A. J. Townsend  
Frease and Bond  
Attorneys

Nov. 19, 1929.

H. M. NAUGLE ET AL.

1,736,324

## STRIPSHEET MANUFACTURE

Filed May 24, 1927

3 Sheets-Sheet 2



Fig. 5



Fig. 6



Fig. 7

## Inventors

By

*H. M. Naugle  
A. J. Townsend*

Frease and Bond Attorneys

Nov. 19, 1929.

H. M. NAUGLE ET AL.

1,736,324

## STRIPSHEET MANUFACTURE

Filed May 24, 1927

3 Sheets-Sheet 3



Fig. 8



Fig. 9

## Inventors

*H. M. Naugle  
A. J. Townsend*

၁၃၁

Frease and Bond Attorneys

## UNITED STATES PATENT OFFICE

HARRY M. NAUGLE AND ARTHUR J. TOWNSEND, OF CANTON, OHIO, ASSIGNEES, BY  
MESNE ASSIGNMENTS, TO THE AMERICAN ROLLING MILL COMPANY, OF MIDDLE-  
TOWN, OHIO, A CORPORATION OF OHIO

## STRIP-SHEET MANUFACTURE

Application filed May 24, 1927. Serial No. 193,937.

The invention relates to the production of stripsheets of steel or iron, having the unlimited length of a strip, the thin gauges of a sheet, and an extraordinary width of from twenty to thirty to forty inches and upwards.

Various methods have been proposed from time to time for producing long strips with thin gauges and sheet widths by longitudinal rolling from slabs or sheet bars, as for instance, the methods disclosed in the Davies Patent No. 674,855, the Cushwa Patent No. 904,605, and the Norton Patent No. 1,108,213, but for one reason or another, the disclosure of such patents has never resulted in a successful or commercial production of stripsheets.

In any event, there is nothing in either one of the Davies, the Cushwa, or the Norton patents, which discloses means and methods for successfully reducing by continuous rolling operations a thick strip to a stripsheet in widths exceeding the common strip mill practice, which has heretofore been limited to widths of from twenty to twenty-five inches.

We have heretofore described the making of stripsheets by the methods disclosed in our prior Patents No. 1,536,028, No. 1,544,028, and No. 1,544,269, but in the first instance, the disclosure does not suggest a width of product exceeding the ordinary strip mill practice, which at that time did not exceed twenty inches, and moreover the method excluded a hot rolling operation and was limited to a rapid cold rolling reduction, followed by a quick annealing; in the second instance the stripsheet product was limited to a width of some eight inches; and in the third instance, the stripsheet product was limited to a long, thin, narrow strip or band.

We have also developed improved methods and apparatus for continuously annealing and pickling stripsheets, and improved methods and apparatus for cold rolling and coiling the same, which are set forth in co-pending applications, and the same are necessary or desirable, and in some cases may be essential, for the successful commercial production of stripsheets; and the purpose of the present improvement is to combine and coordinate methods and apparatus which are

necessary to successfully produce for the first time, a commercial commodity of iron or steel having the length of a strip and the width and gauge of a sheet, and also having the uniform and high ductility which is required for deep drawing and forming operations.

The improved method may begin with a steel slab, and may include a continuous heating furnace, a scale breaker and a slab turn-over for removing scale from the slab, a reversing universal mill for roughing and breaking down the slab to a strip and edge rolling the same, a series of four-high or cluster mills for reducing the strip by single pass to a sheet gauge during the same heat, a continuous blue annealing furnace for heat treating the hot rolled stripsheets; or a continuous pickling apparatus for removing scale from the hot rolled strip sheet, a plurality of four-high or cluster mills for reducing a stripsheet to a finishing gauge by cold rolling operations, and a continuous furnace for quick annealing the finished stripsheet; together with such intermediate coilers, levelling rolls, traveling welders and like apparatus, which may be necessary or desirable for carrying out the more general operations which may be employed.

It will be understood that the hot rolling, the blue annealing or the continuous pickling, the cold rolling and the quick annealing operations may each one follow the other during a continuous movement of a strip without any intervening coiling operations, but such an arrangement of the necessary apparatus for accomplishing the successive operations would extend the same to such a length as would be inconvenient, to say the least, in the operation of a plant; and for that reason, it is preferred to coil the strip at the end of each one of the continuous hot rolling, pickling, cold rolling and annealing operations, and to carry out the alternate operations in reverse directions, so as to bring them all under a common roof of limited length and a reasonable width.

Moreover, by such an arrangement, each strip is wound in a coil at the end of each major operation and may be detained or

stored before proceeding to the next major operation, which gives greater flexibility in the operation of a series of apparatus as a whole and also in the operation of each separate portion thereof.

5 A combination and arrangement of commercial apparatus which has been successfully employed in carrying out the present improvements, is illustrated more or less diagrammatically in the accompanying drawings, forming part hereof, in which—

10 Figure 1 is a plan view of two continuous furnaces, a scale breaker, a slab turn-over, a reversing universal roughing mill, a tandem series of four, four-high mills, together with the intervening conveyer tables, for reducing a slab to a strip sheet by hot rolling operations;

15 Fig. 2, a side elevation of the same; Fig. 3, a plan continuation of the hot rolling apparatus, including a shears for cropping off ends or cutting thicker strips or plates to lengths, a porcupine transfer and piler tables for handling strips or plates cut to length, and a coiler and a turn table for coiling strip sheets and delivering them in a desired direction;

20 Fig. 4, a side elevation of the same; Fig. 5, a plan of a continuous furnace and appurtenances, which may be used for blue annealing strip sheets made solely by hot rolling operations;

25 Fig. 6, a plan view of a continuous pickling apparatus and appurtenances thereto, for removing scale and the like from a hot rolled strip sheet;

30 Fig. 7, a side elevation of the same; Fig. 8, a plan view showing below, a tandem series of four, four-high rolls for cold rolling, reducing and finishing operations, together with two additional mills for special finishing operations; and showing above, a continuous annealing furnace and appurtenances for quick annealing cold rolled and finished strip sheets; and

35 Fig. 9, a side elevation of the same. Similar numerals refer to similar parts throughout the drawings.

40 For carrying out the improved methods, an open hearth ingot may be reduced by a slabbing mill and cut to form slabs, say three inches thick and thirty-six inches wide, and from four to twelve feet in length, according to the desired dimensions of the 45 strip sheet to be produced, and then heated to a rolling temperature.

45 Such slabs may be heated while moving laterally through one of the heating furnaces 12 on to a discharge skid 13, and then be conveyed by a roller table 14<sup>a</sup> to a scale breaker 15 provided with bending rolls having cutting edges, which act to reversely flex the comparatively soft body of the slab and to detach and cut or break the relatively hard 50 surface scale therefrom; whence the slab is

conveyed by roller tables 14<sup>b</sup> and 14<sup>c</sup> over a slab turnover 16 to a roughing mill 17, which may be and preferably is a reversing universal mill, wherein from five to eleven passes breaks down the slab and forms a 55 strip plate of say three-eighths of an inch thick, thirty-six inches wide, and some fifty feet long, depending upon the original length and thickness of the slab.

60 During the roughing operation, the vertical axis rolls in the sides of the universal mill act to edge roll the slab as it is being broken down to a strip plate, to true the edges and define the width of the strip plate; it being understood that this edge rolling is not necessarily done by the rolls of a universal mill, but may be done by any vertical axis rolls acting in conjunction with the roughing rolls.

65 From the roughing mill, the strip is carried by a roller conveyor 14<sup>d</sup> to the first one of a tandem series of say four or more four-high or cluster mills 18<sup>a</sup>, 18<sup>b</sup>, 18<sup>c</sup>, and 18<sup>d</sup>, through which the strip is passed continuously and by which it may be reduced by single 70 ply passes in the immediately succeeding operations of the successive mills to a strip sheet of from eleven to eighteen gauge, thirty-six inches wide and some three hundred feet long, according to the original length and 75 thickness of the slab.

80 A strip sheet thus produced may be conveyed by a roller table 14<sup>e</sup> through automatic shears 19, which may be used for cropping irregular ends of the strip sheet; whence it 85 may be conveyed by a traveling conveyor 14<sup>f</sup> directly to a coiler 20, from which the coil 90 may be delivered on to a turn-table 21 for delivering it either longitudinally or laterally from the end of the hot rolling apparatus, 95 as may be desired.

100 When, however, a strip of from twelve to seven gauge or more in thickness is produced, which does not require annealing or pickling for commercial use, the strip may be cut to 105 length by the automatic shears 19, and a porcupine table 22 may be interposed between the shears and the coiler, for transferring the 110 cut strip to a piler table 23, whence a pile of the same may be carried by a conveyor 14<sup>g</sup> to 115 a place of delivery.

120 When a hot rolled strip sheet is produced with a thickness of from fourteen to eighteen gauge, which is intended for use without a further cold rolling reduction, the grain size may be affected by rolling below the critical temperature, and this so hardens the material as to require an annealing operation to soften the metal to make a ductile commercial commodity. This may be accomplished by a 125 continuous blue annealing operation, which may be carried out in the apparatus diagrammatically illustrated in Fig. 5, which may include a coil table 24, levelling rolls 25, a traveling welder 26, an annealing fur- 130

nace 27, a table 28, pinch rolls 29, and either an automatic shears 30 or a coiler 31, depending upon whether the product is to be cut into lengths or wound in a coil.

When, however, a hot rolled strip or stripsheet is to be further reduced in thickness by a cold rolling operation, it is pickled to remove the scale and other oxidation resulting from the hot rolling reduction, which pickling may be done by the continuous pickling apparatus diagrammatically illustrated in Figs. 6 and 7 of the drawings, and may include a coil holder 32, levelling rolls 33, a traveling welder 34, a pickling tank 35, a water bath 36, an alkali bath 37, pinch rolls 38, and either automatic shears 39, or a coiler 40, depending upon whether the strip is cut to length for use, or wound in a coil for further operations.

The pickled strip or stripsheet is then substantially reduced in thickness to a desired gauge and finish by a cold rolling operation, which may be accomplished by apparatus illustrated in Figs. 8 and 9, and may include a coil holder 41, a tandem series of four, four-high mills 42<sup>a</sup>, 42<sup>b</sup>, 42<sup>c</sup> and 42<sup>d</sup>, and a coiler 43; and the successive rolls and the coiler may be operated at successively increasing peripheral speeds, so as to constantly maintain an elongated stretching tension greater than the elastic limit but less than the ultimate strength of the metal in the stripsheet on the delivery side of the rolls.

Additional stands of four-high mills 42<sup>e</sup> and 42<sup>f</sup>, and coilers 43<sup>e</sup> and 43<sup>f</sup>, as shown in Figs. 8 and 9, may be employed for giving further tempering or finishing passes to the stripsheet, either before or after the same is annealed.

The stripsheet is reduced by the cold rolling operation to the desired gauge and finish, which may be from sixteen to twenty-four gauge or thinner, and it is then given a quick annealing operation by means of apparatus also illustrated in Figs. 8 and 9, which may include a coil holder 44, a leveller 45, a slitter or edge trimmer 46, a traveling spot welder 47, a quick annealing furnace 48, a cooling duct 49, a cleaning trough 50, pinch rolls 51, and either an automatic shears 52 or a coiler 53, depending upon the length of the stripsheet product desired.

The scale breaking operation may be done by the apparatus illustrated in our application for scale breaker filed herewith, Serial No. 193,938; the pickling operation may be carried out by the method and apparatus set forth in our application for continuous pickling processes, filed November 12, 1926, Serial No. 147,878; the cold rolling operations may be carried out by the method and apparatus set forth in our pending application for method of cold rolling and coiling strips, filed April 28, 1927, Serial No. 187,186, and also by the method set forth in our patent for

method of making stripsheets, No. 1,536,028, granted April 28, 1925; the quick annealing operations may be carried out by methods and apparatus set forth in our pending application for continuous annealing and pickling processes, filed July 1, 1925, Serial No. 40,739; the traveling welders used may be of the character set forth in our pending application for welding machines, filed September 18, 1926, Serial No. 136,360; and the automatic shears employed may be of the character set forth in the pending application of Townsend and Miller for automatic shears, filed April 6, 1927, Serial No. 181,410; to which several applications reference is made for detailed descriptions of the various methods and apparatus set forth therein.

In the production of a commercially satisfactory and acceptable stripsheet product in extraordinary widths, it is essential that the scale formed on the slab in the heating furnaces shall be broken and completely and cleanly removed from the sides of the slab prior to the roughing and hot rolling operation, because any portion of the scale however small, which remains on the surface of the slab, will be rolled into the same by the roughing and reducing rolls to such an extent as to cause a rejection of stripsheets containing the same; and it is impossible to remove such scale by a pickling process without producing such deep pits as will destroy the surface thereof, and which cannot be entirely eliminated by a cold rolling operation.

It is also desirable, if not necessary, to accompany the reducing operation of the roughing mill with an edge rolling operation for the purpose of controlling and defining the exact width of the strip prior to the time it is reduced from a plate or strip gauge to a sheet gauge; because the true edges and definite width then given to the strip is so little affected by the subsequent reducing rolling in the hot and cold mills as to be negligible, so that true edges and a substantially definite width in the finished stripsheet is substantially caused by the edge rolling operation in conjunction with the operation of the roughing rolls, and may not require an edge trimming of the stripsheet product.

It is necessary to anneal the thinner strip sheets produced solely by hot rolling operations because, as already stated, the grain size may be affected by rolling below the critical temperature, thus giving the material a hardness which is not satisfactory or acceptable for commercial uses; and the extraordinary length and width of stripsheets requires a heat treatment by a quick continuous annealing process to give a uniformity of grain structure throughout the length and width of the stripsheet, so as to render satisfactory an otherwise unacceptable product.

It is also essential to pickle the stripsheet

- before the cold rolling operation to completely remove therefrom all scale and other oxidation from the surface thereof, which can best be done by a continuous pickling process; and it is also essential to quick anneal a strip after it has been cold rolled to produce the desired gauge and finish, for the purpose of correcting the micro-structure of the metal while preventing an objectionable grain growth therein and a detrimental scale thereon during the annealing operation, and this can only be done by a continuous quick annealing operation, during which the metal is maintained at an annealing temperature during a period of only about one minute, to give the stripsheet a uniform high ductility and clean surface throughout its length and width.

- Finally, each and all of these operations must be performed in a continuous manner to avoid cutting the stripsheet into lengths before the final operation to produce the desired product has been completed; and in this manner is produced, for the first time, a rolled steel commodity having the unlimited length of a strip and the thin gauge and extraordinary width of a sheet, and being uniformly ductile throughout its length and width.

30 We claim:—

1. The method of making a stripsheet from a steel slab which includes heating the slab to a rolling temperature, then completely and cleanly removing all scale therefrom by mechanical means, and then rolling the slab by single ply passes to produce a commercial commodity having the unlimited length of a strip and the width and gauge of a sheet, all without reheating the steel.
- 40 2. The method of making a stripsheet from a steel slab which includes heating the slab to a rolling temperature, then rough rolling the slab to form a strip while edge rolling the same to form true edges and define the width of the strip plate, and then continuously rolling the strip plate by single ply passes to produce a commercial commodity having the unlimited length of a strip and the width and gauge of a sheet with defined edges, all without reheating the steel.

- 50 3. The method of making a stripsheet from a steel slab which includes heating the slab to a rolling temperature, then completely and cleanly removing all scale therefrom by mechanical means, then rough rolling the slab to form a strip plate while edge rolling the same to form true edges and define the width of the strip plate by single ply passes, and then continuously rolling the strip plate to produce a commercial commodity having the unlimited length of a strip and the width and gauge of a sheet with defined edges, all without reheating the steel.

- 60 4. The method of making a stripsheet from a steel slab which includes heating the slab

to a rolling temperature, then rough rolling the slab to form a strip plate, then continuously rolling the strip plate by single ply passes in a plurality of mills to form a stripsheet, all without reheating the steel, and then continuously annealing the stripsheet to produce a ductile commercial commodity having the unlimited length of a strip and the width of a sheet.

5. The method of making a stripsheet from a steel slab which includes heating the slab to a rolling temperature, then rough rolling the slab to form a strip plate, then continuously rolling the strip plate by single ply passes in a plurality of hot mills to form a stripsheet, all without reheating the steel, then continuously pickling the stripsheet to remove oxidation therefrom, and then continuously rolling the stripsheet in a plurality of cold mills to substantially reduce its thickness to the desired gauge and finish, to produce a commercial commodity having the unlimited length of a strip and the width and gauge of a sheet.

6. The method of making a stripsheet from a steel slab which includes heating the slab to a rolling temperature, then rough rolling the slab to form a strip plate, then continuously rolling the strip plate by single ply passes in a plurality of hot mills to form a stripsheet, all without reheating the steel, then continuously pickling the stripsheet to remove oxidation therefrom, then continuously rolling the stripsheet in a plurality of cold mills to substantially reduce its thickness to the desired gauge and finish, and then continuously annealing the stripsheet to produce a uniformly ductile commercial commodity having the unlimited length of a strip and the width and gauge of a sheet.

7. The method of making a stripsheet from a hot strip plate which includes continuously rolling the strip plate by single ply passes in a plurality of hot mills to form a stripsheet without reheating the steel, then continuously pickling the stripsheet to remove oxidation therefrom, then continuously rolling the stripsheet in a plurality of cold mills to substantially reduce its thickness to the desired gauge and finish, and then continuously annealing the stripsheet to produce a uniformly ductile commercial commodity having the unlimited length of a strip and the width and gauge of a sheet.

HARRY M. NAUGLE.  
ARTHUR J. TOWNSEND.

120

125

130